

## UNITED STATES PATENT OFFICE

2,262,696

## METHOD OF TREATING ALUMINUM ALLOYS

Joseph A. Nock, Jr., Tarentum, and Fred Keller, New Kensington, Pa., assignors to Aluminum Company of America, Pittsburgh, Pa., a corporation of Pennsylvania

**No Drawing. Application October 21, 1939, Serial No. 300,658**

7 Claims. (Cl. 148—4)

This invention relates to methods of treating certain aluminum base alloys employed in making articles which will receive an artificial oxide coating, and more particularly relates to the treatment of the alloys to improve their appearance when so coated. The expression "aluminum base alloys" as used herein refers to alloys which contain at least 75 per cent aluminum.

By various chemical and electrochemical processes known in the art—for example, those described in U. S. Patents 1,869,058 and 1,900,472—aluminum and aluminum base alloy surfaces may be provided with an artificially produced coating which consists substantially of aluminum oxide, and which is generally referred to as an "oxide coating." Such oxide coatings are of appreciable thickness as compared with the very thin film of oxide which is normally produced on the surface of aluminum and its alloys by contact with air.

It has been found that when articles of non-heat treatable aluminum base alloys which, at room temperature and under equilibrium conditions, contain undissolved manganese, iron and silicon, or undissolved compounds containing the elements just mentioned (which elements and compounds are referred to hereinafter as "substantially undissolved components"), are provided with an artificially produced oxide coating, whether that coating be produced by a chemical treatment or by an electrochemical treatment, their surface frequently presents a non-uniform appearance, characterized by an irregular pattern of light and dark areas, with the result that the surface has a streaked appearance. Such a streaked appearance is objectionable when the metal is used for purposes where a uniform finish is desirable. By the expression "non-heat treatable aluminum base alloys," as used above and hereinafter, is meant aluminum base alloys which are not susceptible of having their strength substantially improved by a solution heat treatment or by precipitation hardening after a solution heat treatment.

It is an object of our invention to prevent or reduce a streaked appearance in oxide coated surfaces of non-heat treatable aluminum base alloys which contain a substantially undissolved component. It is a further object of our invention to provide a method of treating non-heat treatable aluminum base alloys which contain a substantially undissolved component, which method will prevent or reduce surface streaking of these articles when they receive an artificially produced oxide coating.

We have found that streaks in artificially oxide

coated surfaces of non-heat treatable aluminum base alloys containing a substantially undissolved component can be prevented or reduced. To accomplish this result, the alloy body should preferably be heated for a period of about 1 to 10 hours at a temperature between 1100° F. and the temperature of incipient fusion of the metal, and then cooled to the normal hot working temperature and hot worked. Although it is preferable to subject the body to the high temperature treatment just mentioned before any hot working is done, the high temperature treatment may follow a hot working step. For example, it is possible to heat the metal to the normal hot working temperature and complete any preliminary hot working operations in the usual manner, and then employ the high temperature treatment followed by a final hot working operation as above described. However, it is preferable that only one hot working operation follow the high temperature treatment herein described. Subsequent to the hot working operation which follows the high temperature treatment, the body may be further worked by cold rolling or by any other cold working process to produce the desired final shape which is to receive the artificially produced oxide coating. The benefit of the high temperature treatment persists in the material whether or not it undergoes further fabrication by cold working. The material may also be subjected to an annealing treatment at the temperatures commonly used for that purpose and then cold worked without detrimental effect.

In addition to containing a substantially undissolved component, the metal may also contain other relatively insoluble elements, such as chromium, titanium, zirconium, molybdenum, nickel, or tungsten, and it may also contain soluble ingredients in amounts insufficient to produce precipitation hardening. Examples of non-heat treatable aluminum base alloys which contain a substantially undissolved component, and which are beneficially affected by the treatment described, are those alloys composed of aluminum and from 0.5 to 3 per cent manganese, with or without iron and silicon impurities to a total of between 0.1 and 1 per cent; or aluminum and from 0.5 to 2.5 per cent manganese, and from 0.25 to 2 per cent magnesium, with or without iron and silicon impurities to a total of between 0.05 and 1 per cent; or aluminum and from 0.5 to 2.5 magnesium, from 0.1 to 2 per cent zinc, and from 0.05 to 0.25 per cent copper, plus iron and silicon impurities to a total of between 0.05 and 0.50 per cent; or aluminum and from 1 to 3 per cent mag-

nesium, and from 0.1 to 0.75 per cent chromium, plus iron and silicon impurities to a total of between 0.1 and 0.35 per cent. Within the ranges given, the iron and silicon usually combine to form a substantially insoluble component. Likewise, the iron sometimes combines with other alloying constituents to form insoluble compounds.

The aluminum base alloy body which is subjected to the elevated temperature may be in the form of an ingot or billet, or in any other form which is adapted for hot working. Generally, the most efficient practice is to heat the metal in ingot form because the heating step which is necessary to prepare the metal for hot working may thereby be combined with the high temperature treatment. The maximum temperature to which the metal may be heated will vary in the operation of my process, since the temperature of incipient fusion differs in various alloys. However, it is necessary to use a temperature of at least 1100° F. in order to obtain the desired results. The duration of the heating step also varies, depending upon such factors as the mass of the material being treated, the internal structure, and the composition of the alloy. In the case of a metal of comparatively thin section, for example 1 inch, a period of 2 hours is ordinarily sufficient to prevent any substantial streaking of the oxide coated article; whereas with thicker bodies of metal, it may be necessary to heat them for as long as 10 hours or more to obtain the same results.

In performing the hot working operation which follows the heating step, any type of working process may be used, as, for example, rolling, forging, pressing, or extruding. The hot working temperature to which the metal should be cooled following the heating step will vary with the particular type of working operation employed and the composition of the alloy. For example, in the rolling of an aluminum base alloy containing 1.25 per cent manganese and 1 per cent magnesium, a temperature of about 825° F. is used. In the case of an aluminum base alloy containing 1.25 per cent manganese, the rolling temperature range is about 800 to 900° F., and the usual extrusion temperature range is 700 to 950° F.

Various methods known in the art for cooling hot metal may be used to cool the metal to the hot working temperature, since the rate of cooling is not critical, but it has been found that it is satisfactory to cool the heated body in air, and that method is preferred. It is essential, nevertheless, that the body be cooled to at least a temperature at which hot working can be satisfactorily performed.

Although the best results are obtained if the heated metal is worked before it has cooled below the hot working temperature, beneficial results may also be secured even though the metal is permitted to cool to room temperature and is then reheated to bring it to the working temperature. However, it is preferable that the metal not be permitted to cool below about 650° F. following the high temperature treatment and prior to hot working.

As a specific example of our invention, an ingot of an alloy containing 1.25 per cent magnesium, 0.5 per cent zinc, 0.15 per cent copper, iron and silicon impurities to a total of 0.2 per cent, and the balance aluminum, was heated in a furnace at a temperature of 1125° F. for 4 hours. It was then removed from the furnace and allowed to cool in air to a temperature of

825° F., whereupon it was rolled into slab form. The slab was subsequently annealed and cold rolled to the desired gauge. When the material was given an electrolytically produced oxide coating by making it the anode for 30 minutes in a 15 per cent solution of sulfuric acid at 70° F. and at a current density of 12 amperes per square foot of surface, the surfaces were found to be substantially free of streaks and to have a uniform appearance.

In another instance, an ingot of an aluminum base alloy composition of 1.25 per cent manganese, iron and silicon impurities to a total of about 0.5 per cent, and the balance aluminum was heated at a temperature slightly above 1200° F. for 2 hours, allowed to cool in air to 900° F., and was then hot rolled to slab form. When cold rolled sheet produced from this slab was oxide coated in the manner stated in the preceding paragraph, the surfaces of the metal had a uniform, unstreaked appearance.

We claim:

1. In the art of making artificially oxide coated aluminum base alloy articles, a method for the production of oxide coated surfaces substantially devoid of irregular light and dark areas or streaks comprising the steps of heating at a temperature of at least 1100° F. a body of a non-precipitation-hardening aluminum base alloy containing at least one substantially undissolved component, but below the temperature of incipient fusion of the alloy, for a period of one to ten hours, cooling said body to at least a temperature at which it can be hot worked, hot working said body, and subsequently artificially oxide coating said body.

2. In the art of making artificially oxide coated aluminum base alloy articles, a method for the production of oxide coated surfaces substantially devoid of irregular light and dark areas or streaks comprising the steps of heating at a temperature of at least 1100° F. a body of a non-precipitation-hardening aluminum base alloy which contains at least one substantially undissolved component, but below the temperature of incipient fusion of the alloy, for a period of one to ten hours, cooling said body to at least a temperature at which it can be hot worked, but above 650° F., thereafter hot working said body, and subsequently artificially oxide coating said body.

3. In the art of making artificially oxide coated aluminum base alloy articles, a method for the production of oxide coated surfaces substantially devoid of irregular light and dark areas or streaks comprising the steps of heating at a temperature of at least 1100° F. a body of a non-precipitation-hardening aluminum base alloy which contains at least one substantially undissolved component, but below the temperature of incipient fusion of the alloy, for a period of one to ten hours, cooling said body to the hot working temperature, hot working said body, and subsequently artificially oxide coating said body.

4. In the art of making artificially oxide coated aluminum base alloy articles, a method for the production of oxide coated surfaces substantially devoid of irregular light and dark areas or streaks comprising the steps of heating a body of an aluminum base alloy containing from 0.5 to 2.5 per cent magnesium, from 0.1 to 2 per cent zinc, from 0.05 to 0.25 per cent copper, and from 0.05 to 0.5 per cent iron and silicon, the balance being substantially all aluminum, said

heating operation being conducted at a temperature of at least 1100° F., but below the temperature of incipient fusion of the alloy, for a period of one to ten hours, cooling said body to a temperature above 650° F., hot working said body, and subsequently artificially oxide coating said body.

5. In the art of making artificially oxide coated aluminum base alloy articles, a method for the production of oxide coated surfaces substantially devoid of irregular light and dark areas or streaks comprising heating a body of an aluminum base alloy containing from 0.5 to 3 per cent manganese, the balance being substantially all aluminum, said heating operation being conducted at a temperature of at least 1100° F., but below the temperature of incipient fusion of the alloy, for a period of one to ten hours, cooling said body to a temperature above 650° F., hot working said body, and subsequently artificially oxide coating said body.

6. In the art of making artificially oxide coated aluminum base alloy articles, a method for the production of oxide coated surfaces substantially devoid of irregular light and dark areas or streaks comprising heating a body of an aluminum base alloy containing from 0.5 to

2.5 per cent manganese and from 0.25 to 2 per cent magnesium, the balance being substantially all aluminum, said heating operation being conducted at a temperature of at least 1100° F., but below the temperature of incipient fusion of the alloy, for a period of one to ten hours, cooling said body to a temperature above 650° F., hot working said body, and subsequently artificially oxide coating said body.

10 7. In the art of making artificially oxide coated aluminum base alloy articles, a method for the production of oxide coated surfaces substantially devoid of irregular light and dark areas or streaks comprising heating a body of an aluminum base alloy containing from 1 to 3 per cent magnesium, from 0.1 to 0.75 per cent chromium, and from 0.1 to 0.35 per cent iron and silicon, the balance being substantially all aluminum, said heating operation being conducted at a temperature of at least 1100° F., but below the temperature of incipient fusion of the alloy, for a period of one to ten hours, cooling said body to a temperature above 650° F., hot working said body, and subsequently artificially oxide coating said body.

15 20 25 JOSEPH A. NOCK, JR.  
FRED KELLER.